

# UNITED STATES PATENT OFFICE.

JOHN FREDERICK BRIGGS, OF SPONDON, NEAR DERBY, ENGLAND, ASSIGNOR TO  
AMERICAN CELLULOSE AND CHEMICAL MANUFACTURING COMPANY LIMITED,  
A CORPORATION OF DELAWARE.

## TREATMENT OF CELLULOSE ACETATE PRODUCTS.

1,425,364.

Specification of Letters Patent.

Patented Aug. 8, 1922.

No Drawing.

Application filed April 16, 1921. Serial No. 461,978.

To all whom it may concern:

Be it known that I, JOHN FREDERICK BRIGGS, a subject of the King of Great Britain and Ireland, of Spondon, near Derby, 5 England, have invented certain new and useful Improvements Relating to the Treatment of Cellulose Acetate Products, of which the following is a specification.

This invention relates to the treatment of 10 filaments, threads or fabrics of or containing cellulose acetate, having a lower degree of acetylation than triacetate, with the object of rendering them amenable to dyeing, and to the dyeing of such filaments, threads or 15 fabrics.

The saponification of triacetates of cellulose to remove acetyl groups by treatment with saponifying agents, e. g. heating with alkaline solutions, is generally known, see 20 for instance Cross and Bevan, "Researches on cellulose" 11 (1906) page 11.

As is well known, cellulose triacetates possess but little affinity for dyes, and especially for direct or substantive colours, which is 25 understandable from a consideration of the fact that the hydroxyl groups of the cellulose are blocked by the acetyl groups. One might therefore expect that lower cellulose acetates would show an improved affinity 30 for dyestuffs or dye better than triacetate. It was found that this is to some extent the case, the lower acetates showing an improvement in regard to the number of dyes which can be applied to them. So far as triacetates 35 are concerned, it has been proposed (see for example British Patent 20672 of 1910) to partially saponify the cellulose acetate in threads, fabrics or materials made therewith, in order to render them more amenable to 40 dyeing.

But it has also been found that the lower acetates of cellulose, i. e. which are substantially lower than cellulose triacetate, for instance those in which from 2 to 3 acetyl 45 groups are combined with one molecule of cellulose  $C_6H_{10}O_5$ , cannot be dyed with dyes in general by the ordinary or commercial methods applicable to non-acetylated cellulose; for example they cannot be satisfactorily dyed directly with substantive cotton dyestuffs, and even with basic and acid 50

dyestuffs the possibility of dyeing directly, or with the usual mordants, is restricted to a limited number of dyestuffs.

It is true that the specification of a previous application Serial No. 411805 describes a process whereby cellulose acetate threads or fabrics may be rendered amenable or more amenable, to dyeing with basic, acid, substantive, vat or other dyes by treatment with ammonium thiocyanate or other thiocyanates prior to or during the dyeing operation, and that this process enables the lower cellulose acetates, with an acetyl content below that of cellulose triacetate, to be also satisfactorily dyed.

The object of the present invention is to provide a new process whereby, while substantially maintaining the weight, mechanical strength, dry or wet, and other technical valuable properties of the original cellulose acetate, threads or filaments of any degree of acetylation below triacetyl cellulose and especially of cellulose acetate having a content of combined acetyl corresponding to about  $2\frac{1}{2}$  acetyl groups per molecule of cellulose  $C_6H_{10}O_5$ , these threads, filaments or fabrics made therewith can be rendered capable of dyeing directly or with the use of mordants or other suitable adjuncts, with any dyes, such as substantive dyes, acid or basic dyes, vat dyes or sulphur dyes, which are commercially applicable to equivalent threads or filaments composed of non-acetylated cellulose.

According to the present invention the threads, filaments or fabrics referred to are subjected to a superficial alkaline saponification with a quantity of caustic soda or other alkaline saponifying agent limited to an amount such that the decrease in weight corresponding to the saponification effected thereby is restricted to from about 3 per cent or less to not more than about 10 per cent of the original weight of the cellulose acetate threads or filaments, and preferably to not more than about 5 per cent of this weight, this saponification being effected at temperatures of between about  $60^{\circ}$  and about  $80^{\circ}$  C., and preferably between about  $70^{\circ}$  and  $75^{\circ}$ . Such a process of saponification, while materially maintaining the weight,

strength and other desirable properties of the cellulose acetate threads or filaments, renders them capable of being dyed with any dye such as referred to.

- 5 It is important that the superficial saponification of the cellulose acetate threads or filaments shall not exceed an amount corresponding to a decrease in weight of about 10%, as beyond this amount the cellulose acetate core or interior of the threads or filaments would be attacked to too great an extent to enable the technically valuable properties of the original cellulose acetate threads such as strength, elasticity and weight, to be 10 sufficiently retained. Also the temperature is of importance, because if this is too low the restricted saponification proceeds too slowly and irregularly to permit satisfactory results to be obtained in dyeing. The temperature should therefore not be below 60° C. and it is usually best to work at about 70°-75° C.

- In carrying out the invention the quantity of alkaline saponifying agent is restricted 25 to about the amount corresponding to the extent of saponification required, that is to say, to a quantity such as will give this amount of saponification by its approximately complete exhaustion.
- 30 This provides a reliable method of controlling the extent of the saponification to the desired degree, so as to maintain substantially the weight and other technically valuable properties of the cellulose acetate threads or filaments as mentioned, and render them amenable to dyeing.

- My process of treatment of the said cellulose acetate threads or filaments also provides a means of controlling or grading the 40 depth of shade of the dyeing as hereinafter referred to.

- As saponifying agent, I use in particular caustic alkali, preferably a solution of caustic soda, although it is obvious that the principle of my process may be fulfilled by the use of other known alkaline saponifying agents having similar effects.

- It is desirable that the concentration of the caustic alkali solution employed should 50 not be higher than about 1% and preferably under 0.5%, the best concentration for working being about 0.1%.

- The amount of superficial saponification effected according to the invention corresponds to the employment of from about 55 10% to 3% or less of caustic soda or its equivalent in terms of other alkaline saponifying agents, calculated on the dry weight of the cellulose acetate filaments or goods.
- 60 The range of 10% to 3% will enable full and level shades to be dyed on the cellulose acetate silks.

- When, however, it is desired only to dye the goods to a pale shade, a smaller proportion of caustic soda than that indicated for

full shades may be expended in the saponification.

The loss of weight in the form of saponified acetyl groups which the silk undergoes as the result of the treatment of the invention varies directly with the proportion of caustic soda or other alkaline saponifying agent expended, and can thus be accurately controlled. For practical purposes this loss of weight may be taken as approximately 70 equal to the quantity of caustic soda used up (mol. weight of NaOH=40; mol. weight CH<sub>3</sub>CO minus H=42), that is to say the weight of the acetate filaments, silk or the like, will only decrease to an extent between 75 about 3% or less and about 10% of their original weight, according to the particular dyes used, and the depth of shade to be dyed.

By regulating the amount of the caustic 80 soda or equivalent saponifying agent employed for the process, it is possible to direct or regulate the shade of dyeing according to desire, which is especially important when it is required to dye light or pale 85 shades.

The dyeing of cellulose acetate filaments or threads or goods containing the same, with employment of my saponification process may be performed in any appropriate 90 way according to two methods which I call the "pretreatment method" and the "single bath method."

According to the "pretreatment method" 95 saponification and dyeing are performed in 100 separate operations, which may be either immediately consecutive, or divided by the interposition of other desired operations, which may be chemical, such as scouring, soaping, drying, mordanting or the like, or mechanical such as winding, twisting, knitting, weaving, and like textile operations.

According to the "single bath method" 105 the saponification and dyeing are performed in one bath.

In carrying out the saponification as a separate process I may immerse the goods in a solution containing the predetermined quantity of caustic soda, and heated to the temperature selected for the saponification, and maintain the temperature of the bath, while working the goods about or otherwise taking steps to ensure uniform circulation or penetration of the liquid, until the caustic soda is neutralized or practically so. 110 The treated goods are removed, rinsed, and may be scoured if desired. They may then be passed directly and without drying, to the mordanting or dyeing baths, in which they are treated by known methods similar 115 to those employed for dyeing cotton or cellulose artificial silks. Or else the saponified goods may be dried directly, or after softening with soap solutions, fatty emulsions, or other suitable finishing agents, and passed 120 125 130

through various textile operations before being dyed.

Goods prepared from cellulose acetate filaments which have undergone pretreatment by my process are susceptible to dyeing with any dyes, such as substantive dyes, acid or basic dyes, vat dyes or sulphur dyes, and by any of the methods for example which are practised in the case of artificial 10 silks such as viscose, cuprammonium, and denitrated collodion silks, but they retain special physical qualities, such as superior strength and elasticity in the wet state, which are characteristic of cellulose acetate 15 silk.

In carrying out the saponification as a separate process or pretreatment I may prepare the saponifying bath with hot water to the proportion of 20 to 100 times the 20 weight of cellulose acetate calculated on the dry weight of the goods, and add to this water a measured quantity of concentrated caustic soda solution, sufficient to give the pre-determined restricted proportion of 25 caustic soda on the dry weight of cellulose acetate in the goods. The quantity of water taken is preferably such that the concentration of caustic soda is not less than 0.1% NaOH. Thus, if I am saponifying cellulose acetate silk with 10% of its weight of 30 NaOH, the quantity of water will not be more than 100 times the weight of the cellulose acetate, and if I am saponifying with 5% NaOH, I should not take more than 50 35 times the weight of water on the goods. I may however use other concentrations of soda than those stated, and good results may be obtained by taking water equal to 40 times the weight of cellulose acetate, corresponding to a concentration of 0.25% 40 NaOH, or even 20 times, corresponding to 0.5% NaOH. It is evident that the action is more rapid the higher the concentration, and that if the quantity of water be curtailed, 45 the efficient circulation of the liquor cannot be ensured. I therefore prefer, from a practical point of view, to work with a concentration of about 0.1% NaOH. As before stated, however, the concentration should 50 not be higher than 1%.

The saponifying bath containing the soda is preferably first heated up to the maximum temperature of saponification which should not exceed about 80° C. I generally 55 work at a maximum temperature of 75° C., but I do not confine myself to this temperature, since it is possible to work less rapidly at 60° C.

If the cellulose acetate goods be contaminated with oily stains, so that scouring treatment is required, this may either be given before the goods are entered into the saponifying bath, or with advantage, soap may be incorporated with the caustic soda 60 in the saponifying bath in order to effect

the cleansing and saponification simultaneously.

*Example of pretreatment.*—For the pretreatment of 10 lb. of cellulose acetate silk, I make up a bath with 100 gallons of water 70 at 75° C., adding concentrated caustic soda lye equivalent to 1 lb. of dry NaOH. The silk is entered into this bath without previous wetting, and is quickly immersed and moved through the liquid or the liquid circulated through the silk, so as to ensure homogeneous distribution of the caustic alkali on the silk. The temperature is maintained at approximately 70-75° during the process, care being taken as far as possible 75 to avoid contact of the silk with the heated surface of the vessel. Under the conditions described, the neutralization of the soda and external saponification of the filaments, will be substantially complete within about 45 80 minutes. The treated silk is withdrawn and rinsed; it may be scoured in dilute acetic or other acid if desired, and then passed through a finishing bath containing soap or other suitable softening agent, and dried. 85 Alternatively, it may be passed directly from the pretreatment to the dyeing process without drying, and is there treated in the same manner as other artificial silks. Or it may, directly after the pretreatment be 90 washed and dried and subjected to the usual textile operations and only afterwards dyed; according to requirements.

In the treatment of union or mixed fabrics composed of cellulose acetate silk and 100 cotton, or other fibre, such as natural silk, wool, etc., I calculate the caustic soda employed only on the weight of cellulose acetate present in the goods.

With the single bath method any dyes 105 may be used which bear the presence of alkali in the bath, which is the case with the entire range of direct or substantive cotton dyestuffs, the sulphur dyestuffs and the vat dyestuffs for example. In this method a 110 known and restricted amount of caustic soda, calculated on the dry weight of the cellulose acetate in the goods is added to the dyebath, which is preferably heated up to the desired saponification temperature before the goods are entered. In this case saponification and dyeing of the cellulose acetate threads or goods proceed simultaneously until the predetermined amount of 115 saponifying agent has been exhausted, after which dyeing is continued if necessary until the desired shade is reached. Such a method is particularly favourable for the even dyeing of pale shades, since the initial resistance of the cellulose acetate is only gradually 120 overcome by the saponifying action of the caustic soda, and the dyestuff is therefore prevented from "rushing" on to the fibre. The single bath process is, however, equally 125 applicable to the dyeing of full shades, even 130

when the velocity of saponification exceeds that of the absorption of the dyestuff, by continuing the treatment until both the alkali and the dyebath are exhausted.

5. In carrying out the single bath process, I may, by way of example, make up a saponification bath in the same manner as for the pretreatment process, but adding the desired dyestuff, for instance the requisite quantity 10 of a solution of a substantive cotton dyestuff. The acetate silk is then entered dry into the combined saponifying and dyeing bath at a suitable temperature, say for instance 70° C. to 75° C., and the dyeing is 15 conducted by working the goods in the usual manner. The dyestuff solution may be added in portions at various stages of the process in the manner frequently adopted in dyeing artificial silk, and the rate of exhaustion of the dyebath may be controlled by the addition of known suitable adjuncts, such as soap, in order to promote level dyeing and penetration, or common salt to facilitate the exhaustion of the dyestuff when 20 dyeing full shades, and so forth. If the dyeing is continued after the caustic soda is substantially exhausted, the temperature of the dyebath may be allowed to fall if desired.

6. What I claim and desire to secure by Letters Patent is:—

1. Process for the treatment of threads or filaments of cellulose acetate lower than triacetyl cellulose, or of fabrics of or containing the same, said process consisting in subjecting said goods in an aqueous bath to saponification at a temperature between about 60° and about 80° C. with a quantity of alkaline saponifying agent capable only of effecting by its exhaustion an amount of saponification corresponding to not more than about 10 per cent of the original weight of the cellulose acetate threads or filaments, whereby dyeing of the cellulose acetate goods is facilitated while substantially maintaining their weight and mechanical strength.

2. Process for the treatment of threads or filaments of cellulose acetate lower than triacetyl cellulose, or of fabrics of or containing the same, said process consisting in subjecting said goods in an aqueous bath to saponification at a temperature between about 70° C. and about 75° C. with a quantity of alkaline saponifying agent capable only of effecting by its exhaustion an amount of saponification corresponding to from about 3 to 5 per cent of the original weight of the cellulose acetate threads or filaments.

3. Process for the treatment of threads or filaments of cellulose acetate lower than triacetyl cellulose, or of fabrics of or containing the same, said process consisting in sub-

jecting said goods in an aqueous bath to 65 saponification at a temperature between about 60° and about 80° C. with a quantity of alkaline saponifying agent capable only of effecting by its exhaustion an amount of saponification corresponding to not more 70 than about 10 per cent of the original weight of the cellulose acetate threads or filaments, the alkaline saponifying agent being employed in a concentration not higher than about 1 per cent. 75

4. Process for the treatment of threads or filaments of cellulose acetate lower than triacetyl cellulose, or of fabrics of or containing the same, said process consisting in subjecting said goods in an aqueous bath to 80 saponification at a temperature between about 70° and about 75° C. with a quantity of alkaline saponifying agent capable only of effecting by its exhaustion an amount of saponification corresponding to not more 85 than about 10 per cent of the original weight of the cellulose acetate threads or filaments, the alkaline saponifying agent being employed in a concentration of between about 0.1 per cent and about 0.5 per cent. 90

5. Process for the treatment of threads or filaments of cellulose acetate lower than triacetyl cellulose, or of fabrics of or containing the same, said process consisting in subjecting said goods in an aqueous bath to 95 saponification at a temperature between about 60° and about 80° C. with caustic soda employed in an amount not exceeding about 10 per cent calculated on the dry weight of the cellulose acetate, substantially as and 100 for the purpose described.

6. Process for the treatment of threads or filaments of cellulose acetate lower than triacetyl cellulose, or of fabrics of or containing the same, said process consisting in subjecting said goods in an aqueous bath to saponification at a temperature between about 60° and about 80° C. with caustic soda employed in an amount of from about 3 to about 5 per cent, calculated on the dry weight of the cellulose acetate, substantially 105 as and for the purpose described. 110

7. Process for the treatment of threads or filaments of cellulose acetate lower than triacetyl cellulose, or of fabrics of or containing the same, said process consisting in subjecting said goods in an aqueous bath to saponification at a temperature between about 70° C. and about 75° C. with caustic soda employed in an amount of from about 115 3 to about 5 per cent calculated on the dry weight of the cellulose acetate, substantially as and for the purpose described. 120

8. Process for the treatment of threads or filaments of cellulose acetate lower than triacetyl cellulose, or of fabrics of or containing the same, said process consisting in subjecting said goods in an aqueous bath to 125

- saponification at a temperature between about 60° and about 80° C. with caustic soda employed in an amount of from about 3 to about 5 per cent calculated on the dry weight of the cellulose acetate, the caustic soda being employed in a concentration not higher than about 1 per cent, substantially as and for the purpose described.
9. Process for the treatment of threads or filaments of cellulose acetate lower than triacetyl cellulose, or of fabrics of or containing the same, said process consisting in subjecting said goods in an aqueous bath to saponification at a temperature between about 70° C. and about 75° C. with caustic soda employed in an amount of from about 3 to 5 per cent calculated on the dry weight of the cellulose acetate, the caustic soda being employed in a concentration of between about 0.1 per cent and 0.5 per cent, substantially as and for the purpose described.
10. In a process for the treatment of threads, filaments or fabrics of or containing cellulose acetate lower than triacetyl cellulose by subjection to partial saponification at temperatures between about 60° and about 80° C. with a quantity of alkaline saponifying agent capable only of effecting a saponification corresponding to not more than about 10 per cent of the weight of the cellulose acetate, regulating the amount of the alkaline saponifying agent for the purpose of regulating shades of dyeing, substantially as hereinbefore referred to.
11. Process for the treatment of threads or filaments of cellulose acetate lower than triacetyl cellulose, or of fabrics of or containing the same, said process consisting in subjecting said goods in an aqueous dye bath to saponification at a temperature between about 60° and about 80° C. with a quantity of alkaline saponifying agent capable only of effecting by its exhaustion an amount of saponification corresponding to not more than about 10 per cent of the original weight of the cellulose acetate threads or filaments, whereby dyeing of the cellulose acetate goods is facilitated while substantially maintaining their weight and mechanical strength.
12. Process for the treatment of threads or filaments of cellulose acetate lower than triacetyl cellulose, or of fabrics of or containing the same, said process consisting in subjecting said goods in an aqueous dye bath to saponification at a temperature between about 70° and 75° C. with caustic soda employed in an amount of from about 3 to about 5 per cent calculated on the dry weight of the cellulose acetate, substantially as and for the purpose described.

In testimony whereof I have hereunto subscribed my name.

JOHN FREDERICK BRIGGS.